

May 28, 1968

T. W. HAMBY, JR., ETAL

3,385,363

METHOD FOR METAL COATING A TUBING STRING IN SITU IN A WELL

Filed Sept. 14, 1966



INVENTORS:

TYLER W. HAMBY, JR.

EDWIN A. RICHARDSON

ROBERT N. TUTTLE

BY: *J. H. M. Cartay*  
THEIR AGENT

## 1

3,385,363

## METHOD FOR METAL COATING A TUBING STRING IN SITU IN A WELL

Tyler W. Hamby, Jr., Edwin A. Richardson, and Robert N. Tuttle, Houston, Tex., assignors to Shell Oil Company, N.Y., a corporation of Delaware

Filed Sept. 14, 1966, Ser. No. 579,432  
10 Claims. (Cl. 166—38)

This invention relates to injection wells for thermally treating a subsurface earth formation and more particularly to a method for preventing failure of the casing or a casing-cement bond in an injection oil well.

The producing formations of many oil fields contain low-gravity oil whose viscosity is of a value sufficiently high to prevent easy flow of the oil from the formation and into a well. In some fields of this type, steam soaking of the producing formation is carried out through one or more injection wells in order to reduce the viscosity of the production fluid and drive the heated oil to adjacent wells, in the same field, through which it is produced to the surface.

A typical method for treating an oil-bearing formation by steam injection is disclosed in U.S. Patent No. 3,259,186 to Dietz. In methods of this type an oil well is provided with a casing extending from the top of the well down to at least the top of the producing formation and generally below the producing formation in order to line the well. Tubing string is mounted concentrically within the casing and the casing is perforated in the area of the oil-bearing formation to permit steam to escape into the formation. Due to high temperature of the steam flowing down the tubing string into the formation radiation heat loss from the tubing string increases the casing temperature. The rise in casing temperature can cause destructive axial thermal stresses to be exerted on the casing. Such operations have resulted in severe casing damage in some injection wells, or rupture or cracking of cement holding the casing in the well. In addition, the heat lost to the casing reduces the available heat introduced into the oil-producing formation and thus reduces the efficiency of the thermal recovery process. Laboratory and field tests have shown that the casing temperature during steam injection often exceeds the theoretical maximum allowable casing temperature and has resulted in casing failures in some thermal well installations. It has been estimated that 90% of the heat transfer from the tubing string to the surrounding casing is by radiation.

It is therefore a primary object of the present invention to reduce the radiant heat loss of the tubing string carrying the steam to the oil-bearing formation.

Another object is to reduce the radiant heat loss by coating the tubing with a bright reflective material.

Another object of the present invention is to provide a method whereby the tubing and interior of the well casing are metal-plated in situ.

Still another object of the present invention is to provide a method to increase the available heat injected into the oil-bearing formation to improve the thermal recovery process.

These and other objects of the invention will be understood from the following description taken with reference to the drawing which diagrammatically illustrates a steam injection well installation in cross-section to which the present invention is adaptable.

Referring to the drawing, an injection well casing 10 is cemented in the well in any suitable manner well known in the art. A tubing string 15 is suspended concentrically within the well casing 10 and extends from the surface of the earth down to a point in the lower end of the casing 10 in the area of an oil-bearing formation 22.

## 2

Perforations 16 are provided in the casing 10 which permit the introduction of steam from the tubing string into the formation.

The top of the well installation is closed in any suitable manner. For example, in the arrangement shown, a casing head closure in the form of a flange 18 is welded to the casing 10 to close the annular space 11 between the casing 10 and the tubing string 15.

It will be readily understood that in the thermal recovery apparatus thus far described, the radiant heat loss from the tubing string 15 during steam injection through the tubing string raises the temperature of the casing 10 an undesirable amount.

In accordance with this invention, the radiation heat loss from the tubing string 15 to the casing 10 can be significantly reduced by bright plating the tubing string with a reflective metallic material thereby reducing the tubing emissivity. It has been discovered that the tubing string can be effectively plated by contacting the tubing string with an electroless metal-deposition solution. The electroless metal-deposition can be accomplished by contacting the tubing string with a metal-deposition solution containing chemicals inclusive of metal ions together with a reducing agent which effects a chemical-reduction deposition of metal on the tubing string. This reaction is carried out under subsurface well conditions of temperature and pressure.

The metal plating compound can be a polyvalent metal compound of which the preferred are nickel, cobalt, copper, iron compounds and mixtures thereof, e.g., nickel and/or cobalt chloride, sulfate and/or nitrate and these metal compounds are reduced by such reagents as hypophosphorous acid, hypophosphites, e.g., sodium hypophosphite or alkaline solution of molybdenate, formate and/or hydroxy carboxylates, e.g., hydroxyacetate. The concentration of the metal-containing compounds and the reducing agents in aqueous solutions can be varied over a wide range such as from 1 to 50%, respectively and preferably from 5 to 40% each.

To control hydrogen evolution to a minimum as a result of the reaction, the reducing agents in the metal-plating solutions should be kept at a minimum generally not in excess of 10% of the total electroless metal plating solution particularly when the solutions are alkaline.

Also, hydrogen evolution can be effectively suppressed and the life of the metal-plating reaction increased by addition to such aqueous solutions buffering and chelating agents such as hydroxy carboxylic acids and polycarboxylic acids and their salts, e.g., citric, tartaric, maleic, gluconic, succinic acids or ammonium or alkali metal salts of said acids such as sodium citrate, sodium succinate and the like. However, the gas can be effectively eliminated from the area being metalized by applying pressure of 200 pounds per square inch or more on the system.

When using a hypophosphite as the reducing agent its concentration should be controlled since, depending in part on the phosphorous content of the solution, the metal being deposited can be in the form of an alloy of metal-phosphorous nickel phosphide. High concentration such as above 10% of hypophosphite in the metal-plating solution tends to form these alloys.

Prior to plating the tubing string 15 it is preferable to clean the surface of the tubing string to remove any paint or foreign material. A suitable acid or solvent may be injected into the annular space 11 through access pipe 12 to accomplish this purpose. One method employed for contacting the tubing string with either the cleaning agent or the metal-plating compound to be subsequently injected is to fill the annular space 11 with the fluid, let it stand and then evacuate the annular space

with suitable pumping or pressure means or by opening 5  
expansible packer 14 and draining the fluid into the  
formation 22. Alternatively, the packer can be left open  
and the fluid continuously flushed through the annular  
space 11 thus establishing flowing contact with the  
tubing string. The particular type of packer employed  
is not critical to the invention since many expansible  
packers are available and known in the art which can be  
remotely opened from the top of the well to permit draining  
10 by retracting the packer away from the casing wall. In  
some wells, due to the pressure existing in the formation  
22, it may be necessary to pressurize the annular space  
11 to force the solutions into the formation.

After the surface of the tubing string has been prepared  
15 an aqueous solution containing one of the above-mentioned  
metal-plating compounds and one of the reducing  
compounds is prepared. The solution is then introduced  
into the well by one of the two methods referred to  
above, i.e., by filling the annular space 11 or by flushing  
20 the solution through the annular space. With either method,  
the solution must stay in contact with the tubing string  
a sufficient time to permit the metallic component to de-  
posit on the surface of the tubing string. The reaction  
rate of metal deposition is affected by temperature and  
25 for best results the solution should be introduced into  
the well at a temperature between ambient and 200° F.;  
preferably between 100° F. and 190° F.

After contacting for a sufficient time, the solution is  
drained into the formation past packer 14 or evacuated  
30 by suitable means not shown. Of course, if the drains 13  
are kept open the plating solution is continuously drained  
into formation 22. In addition, gas pressure may be  
supplied to the upper end of the annular space to drive  
the solution into the formation or back up the inside of  
35 the tubing string 15.

During the procedure thus described, it will be observed  
40 that the interior of the casing 10 will also become metal-  
lized as well as any other ferrous surfaces the solution  
may come into contact with, e.g., the interior of the tubing  
string 15. This additional bright coating is desirable  
45 since it further reduces radiant heat loss from the tubing  
string to the casing 10. Other arrangements may be em-  
ployed without departing from the spirit of the invention.  
For example, the lower end of the tubing string could be  
plugged and the string provided with a selectively opened  
50 port to place the interior of the tubing string 15 in com-  
munication with the annular space 11. The plating solution  
could then be introduced through the tubing string 15,  
thus plating the interior of the tubing string as well.

In the preferred method described above, it is assumed  
55 that the tubing string is made of steel. If a non-ferrous  
material is employed, it is necessary to pretreat the tubing  
with an activating agent since the metallic component  
will not deposit on most non-ferrous materials. Palladium-  
activator solutions or stannous-activator solutions and/or  
60 hydrazine-activator solutions can be used, e.g., a palladium  
chloride solution and/or stannous chloride solutions can be  
used for mixtures thereof.

In addition, when an activator is used and drained into  
65 the formation 22, the activator will also contact any un-  
consolidated sand. If the plating solution used to plate  
the tubing string 15 is subsequently drained into the  
formation, the sand particles become metal-plated to form  
a permeable, consolidated formation thus preventing col-  
lapsing or sloughing of the formation. This result is  
70 particularly beneficial since it obviates the separate step  
of consolidating the formation when necessary, by known  
methods, e.g., thermally fusing the formation or using a  
resinous binder) while at the same time accomplishing  
the primary objective of bright coating the tubing string  
75 to reduce its emissivity.

We claim as our invention:

1. A method of bright coating a ferrous tubing string  
within a well comprising:

positioning said tubing string within said well;

mixing an aqueous solution of a metal-plating com-  
pound and a reducing agent;  
introducing into said well said aqueous solution con-  
taining said metal-plating compound and said reduc-  
ing agent; and  
contacting said tubing string with said solution at well  
temperature for a time sufficient to metal-plate said  
tubing string.

2. The method according to claim 1 including the step  
of first contacting said tubing string with a cleaning solution  
to remove foreign material therefrom.

3. The method according to claim 1 including the  
steps of:

lining said well with a ferrous casing; and  
contacting the interior surface of said casing with said  
aqueous solution at well temperature for a time suffi-  
cient to metal-plate said surface.

4. The method according to claim 3 including the step  
of:

providing a packer between said casing and said tubing  
string near the lower end of said tubing string prior  
to introducing said solution into said well, whereby  
a chamber for receiving said solution is formed by  
said casing, packer and tubing string.

5. The method according to claim 3 wherein:  
said metal-plating compound is selected from the group  
consisting of inorganic nickel, cobalt, copper and iron  
compounds.

6. The method according to claim 5 wherein:  
said reducing agent is selected from the group consist-  
ing of hypophosphorus acid, alkali metal hypophos-  
phite, alkali metal molybdate and mixtures there-  
of.

7. The method according to claim 3 wherein:  
said metal-plating compound comprises nickel chloride;  
said reducing agent comprises sodium hypophosphite;  
and  
said aqueous solution is introduced into said well at  
a temperature of 100° F.-200° F.

8. A method of bright coating a tubing string within  
a well comprising:

(a) introducing into said well a first aqueous solution  
containing an activating agent;  
(b) contacting said tubing string with said first solu-  
tion for a time sufficient to activate the surface of  
said tubing string to a form that may be readily plated  
by a metal plating compound;  
(c) introducing into said well a second aqueous solu-  
tion containing a metal plating compound and a re-  
ducing agent into said well; and  
(d) contacting said tubing string with said second  
aqueous solution for a time sufficient to metal plate  
said tubing string.

9. The method according to claim 8 wherein:  
said activating agent is a compound selected from the  
group consisting of palladium and stannous chlorides,  
bromides, nitrates and sulfates and mixtures thereof;  
said metal-plating compound is selected from the group  
consisting of inorganic nickel, cobalt, copper and iron  
compounds; and  
said reducing agent is selected from the group consist-  
ing of hypophosphorus acid, alkali metal hypophos-  
phite, alkali metal molybdate and mixtures there-  
of.

10. The method according to claim 8 wherein steps  
(a) and (c) are performed simultaneously.

#### References Cited

#### UNITED STATES PATENTS

|           |        |         |       |         |
|-----------|--------|---------|-------|---------|
| 1,096,636 | 3/1914 | McIlroy | ----- | 204-26  |
| 2,084,209 | 6/1937 | McIlroy | ----- | 138-145 |
| 3,142,336 | 7/1964 | Doscher | ----- | 166-11  |